

## UNITED STATES PATENT OFFICE

1,927,161

## COLORATION OF MATERIAL

George Holland Ellis, Henry Charles Olpin, and  
William Bertram Miller, Spondon, near Derby,  
England, assignors to Celanese Corporation of  
America, a corporation of Delaware

No Drawing. Application September 27, 1932,  
Serial No. 635,042, and in Great Britain October  
9, 1931

## 9 Claims. (Cl. 8—5)

This invention is a continuation in part of the invention of prior U. S. application S. No. 424,442 filed 29th January, 1930 and relates to the coloration of textile materials made of or containing 5 organic derivatives of cellulose.

U. S. application S. No. 424,442 describes the production of black shades on materials made of or containing cellulose acetate or other cellulose esters or ethers by the oxidation thereon of aniline in the presence of mineral acid in quantity chemically equivalent thereto, there being present in addition a quantity of a substance having an acid reaction, for example a mineral or organic acid, or an acid salt, or a salt having an 10 acid reaction, but preferably an organic acid. By padding a cellulose acetate fabric with a liquor made up with aniline hydrochloride, acetic acid, and the necessary additions, and subsequently ageing, full "ungreenable" black shades of a 15 quality leaving little to be desired may be obtained with great ease.

We have now found that as the additional acid reacting substance formic acid has pre-eminent advantages over organic acids in general, especially when it is desired to apply the coloration by printing or other methods of application involving the use of thickened preparations.

According to the present invention therefore 20 formic acid is employed as the organic acid in the production of black colorations by the process of U. S. application S. No. 424,442.

The present invention is of particular value in 25 that it enables the easy production of full aniline black prints on materials made of or containing cellulose acetate or other esters or ethers of cellulose.

In carrying the invention into effect the aniline and equivalent quantity of mineral acid may 30 conveniently be applied to the materials in the form of mineral acid salts of aniline. There may, for example, be applied to the materials by printing or other means of local application thickened compositions containing the aniline salt, e. g. the hydrochloride or nitrate, and also containing 35 formic acid and an oxidizing agent, for example a chlorate with or without oxidation catalysts such as salts of vanadium, copper, or iron. After 40 printing and drying, the materials may be aged, chromed and soaped according to the usual methods when full "ungreenable" black pattern effects are obtained. Again the materials may 45 be padded with a solution or liquor containing the aniline salt, formic acid and an oxidizing agent, with or without other substances such as 50 catalysts. After padding and drying the mate-

rials are aged, chromed and soaped when excellent full blacks are obtained. The invention is not, however, limited to the application of the aniline salt, formic acid and oxidizing agent by padding or printing, nor to the application of 60 these substances in a single operation. For example, the aniline salt, formic acid and oxidizing agent may be applied by a simple passage of the material through a bath containing them, or they may be applied in succession by padding the 65 material with, or passing the material through, two or more solutions each containing one or more of the necessary compounds. Furthermore, other substances having an acid reaction whether inorganic or organic may be employed in addition to formic acid and mineral acid equivalent to the aniline. Thus, for example, acetic, glycollic, or lactic acids or any of the acidic bodies used in the production of aniline blacks in U. S. application S. No. 424,442 may be employed together with formic acid in the process of the 75 present application.

When dyeing cellulose ester or ether materials in black shades according to the present invention, white or colored pattern effects may be 80 simultaneously produced thereon. Thus for example pattern effects may be produced on the material according to any of the processes mentioned in U. S. application S. No. 424,442.

The following examples illustrate the present 85 invention without in any way limiting it:—

## Example 1

A solution containing:

|                                      | Parts |
|--------------------------------------|-------|
| Aniline salt                         | 15    |
| Formic acid                          | 3     |
| Methylated spirits                   | 12    |
| Gum arabic 1:1                       | 70    |
| is mixed with a solution containing: | 95    |
| Sodium chlorate                      | 9.6   |
| Cupric chloride                      | 0.4   |
| Water                                | 10.0  |
|                                      | 120.0 |
|                                      | 100   |

and immediately printed on to a cellulose acetate fabric by means of a roller having a suitable design. The material is then dried, aged for 3 to 4 minutes in dry steam in a Mather and Platt ager, 105 and then further treated in a bath containing 5 grams per litre of sodium bi-chromate and 5 ccs. per litre of glacial acetic acid at 50° for 5 minutes. After this treatment the material is rinsed, soaped for 10 minutes at 60° C. and 110

2  
finally rinsed and dried when full "ungreenable" black pattern effects are obtained.

Example 2

5 A solution containing:

|                                      | Parts |
|--------------------------------------|-------|
| Aniline salt                         | 20    |
| Methylated spirits                   | 16    |
| Formic acid                          | 4.4   |
| 10 Oleyl diethyl-ethylene diamine    | 0.08  |
| Gum arabic 2: 1                      | 58    |
| is mixed with a solution containing: |       |
| Sodium chlorate                      | 12.8  |
| Cupric chloride                      | 0.64  |
| 15 Water                             | 7.76  |

and immediately applied to a woven fabric consisting of cellulose acetate. The material is then treated according to the method described in 20 Example 1 when a full "ungreenable" black is obtained.

Example 3

A cellulose acetate fabric is padded with a 25 solution containing:

|                                | Parts |
|--------------------------------|-------|
| Aniline salt                   | 12.50 |
| Sodium chlorate                | 9.60  |
| Methylated spirit              | 10.00 |
| 30 Cupric chloride             | 0.40  |
| Oleyl diethyl-ethylene diamine | 0.05  |
| Formic acid                    | 2.75  |
| Water                          | 64.50 |

35 the conditions being so regulated that the fabric retains its own weight of padding liquor. It is then aged for 5-7 minutes in dry steam in a Mather & Platt "ager" and further treated according to the method described in Example 1 40 when a full "ungreenable" black is obtained.

While the invention has been described more particularly in connection with the coloration of materials made of cellulose acetate, it is also applicable to the coloration of materials made of 45 or containing other cellulose esters, for example, cellulose formate, cellulose propionate, or cellulose butyrate, or the products obtained by the treatment of alkalized cellulose with esterfying agents, e. g. the product known as "immunized" 50 cotton obtained with para toluene sulpho chloride, or of cellulose ethers for instance methyl, ethyl or benzyl cellulose, or the products obtained by the reaction of cellulose and glycols or other polyhydric alcohols, or made of or containing 55 mixtures of two or more of these products. The invention may also be applied to the dyeing or otherwise coloring of materials containing one or more cellulose esters or ethers in admixture with a material or materials of another kind, for example cellulosic filaments, but particularly animal fibres such as wool or natural silk. A material containing cellulose acetate and cotton may for example be dyed a solid black in accordance with the present invention.

65

What we claim and desire to secure by Letters Patent is:—

1. Process for the production of black shades on materials comprising an organic derivative of cellulose, comprising oxidizing aniline thereon in the presence of mineral acid in quantity at least chemically equivalent to the aniline and in the presence of formic acid. 80

2. Process for the production of black shades on materials comprising cellulose acetate, comprising oxidizing aniline thereon in the presence of mineral acid in quantity at least chemically equivalent to the aniline and in the presence of formic acid. 85

3. Process for the production of black shades on materials comprising an organic derivative of cellulose, comprising oxidizing aniline thereon in the presence of mineral acid in quantity chemically equivalent to the aniline and in the presence of formic acid. 90

4. Process for the production of black shades on materials comprising cellulose acetate, comprising oxidizing aniline thereon in the presence of mineral acid in quantity chemically equivalent to the aniline and in the presence of formic acid. 100

5. Process for the production of black pattern effects on materials comprising an organic derivative of cellulose, comprising the oxidation of aniline present locally on the materials in the presence of mineral acid in quantity at least chemically equivalent to the aniline and in the presence of formic acid. 105

6. Process for the production of black shades on materials comprising an organic derivative of cellulose, comprising printing the materials 110 with compositions containing aniline and oxidizing the aniline in the presence of mineral acid in quantity chemically equivalent thereto and in the presence of formic acid.

7. Process for the production of black shades on materials comprising cellulose acetate, comprising printing the materials with compositions containing aniline and oxidizing the aniline in the presence of mineral acid in quantity chemically equivalent thereto and in the presence of 120 formic acid.

8. Process for the production of black shades on materials comprising an organic derivative of cellulose, comprising applying to the materials a composition containing aniline and an oxidizing 125 agent, and effecting oxidation in the presence of mineral acid in quantity at least chemically equivalent to the aniline and in the presence of formic acid.

9. Process for the production of pattern effects 130 on materials comprising cellulose acetate, comprising printing the materials with a composition containing aniline, mineral acid in quantity chemically equivalent to the aniline, formic acid, and a chlorate, and ageing to effect oxidation of 135 the aniline.

GEORGE HOLLAND ELLIS.  
HENRY CHARLES OLPIN.  
WILLIAM BERTRAM MILLER.

140

70

145

75

150